

## UNITED STATES PATENT OFFICE

2,390,695

## METHOD OF TREATING PAPER STOCK

John C. Dean, Douglaston, and Roy T. Edwards,  
New York, N. Y., assignors to Socony-Vacuum  
Oil Company, Incorporated, a corporation of  
New York

No Drawing. Application April 25, 1942,  
Serial No. 440,488

4 Claims. (Cl. 92—1.6)

This invention relates to a process for removing ink and pitch from paper pulp or waste paper in the beater stage.

Many types of paper are manufactured partially or entirely of waste paper. This paper, in many instances, has been printed upon with conventional printing inks. Since most inks are black, the presence of the pigment tends to throw the reworked stock off-shade to a pronounced dirty gray color. This is frequently objectionable, and for that reason, steps are often taken to remove the ink during the reworking operation. A further objection is that the presence of the ink in the waste paper may complicate subsequent paper making operations. Foaming difficulties are frequently encountered, and are often attributed to the presence of rosin in the printing ink. Expensive foam control measures must then be taken, or the ink must be removed.

Present methods of de-inking are crude and only partially effective. The most widely used is extraction with kerosene. This solvent is added to the reworked stock in the beater after it has been thoroughly wet-back and broken down to a uniform pulp. Beating is continued until the solvent is completely dispersed throughout the pulp. The pulp is then washed to remove solvent and ink, but complete removal is impossible due to the affinity of the pulp for the mixture. The net effect of this method is to distribute the ink more uniformly, and also to complicate paper making by the presence of objectionable kerosene vapors.

Recourse has been made to the use of emulsifiers to assist in this removal. Attempts have been made to utilize a blend of solvent and emulsifier. Such blends might be termed "emulsifiable solvents," since on addition to water an emulsion of solvent in water is formed. Experiments have shown that they are ineffective, due to the fact that the droplets of solvent are completely surrounded with water, and are prevented from mixing with the water-insoluble inks in the pulp. Consequently, ink removal is poor, and in fact, is less than with straight solvent. An alternate procedure is to add emulsifier to a beater which has been treated with straight solvent. This method is more effective than either of the above, but fails chiefly due to the inability of the emulsifier to completely remove solvent and ink which is firmly bound to the paper fibres. Large quantities of solvents will scour the pulp satisfactorily, but the cost is prohibitive, and the pulp is softened and thus degraded.

Pitch removal from virgin pulp is analogous

to the de-inking of waste paper. Chemical pulp-making processes extract considerable quantities of naturally occurring resins from the pulp, but in few instances result in a pitch-free stock. For many grades of paper, contamination of the cellulose with small quantities of pitch is not objectionable. Such instances include grades sized with from  $\frac{1}{4}\%$  to 3% or over of rosin. However, in the manufacture of tissue papers and other unsized or lightly sized grades, pitch is objectionable. It tends to deposit upon the screens and rolls of the paper machine, and causes imperfect formation and frequent shutdowns for removal. Pitch troubles are combatted by the addition of solvents, such as de-odorized kerosene, to the stock to prevent agglomeration of the pitch, or by the use of small amounts of alum to set the resin firmly on the fibres.

This invention has for its object the provision of an effective method capable of removing ink, pitches, resin, and similar materials from paper stocks. A particularly important object is the provision of an effective process for de-inking recovered paper stocks under conditions economically permitting the attainment of a high color in the finished stocks.

This invention is based upon a novel process using a product applicable for the de-inking of waste paper and the removal of pitch from paper pulp. The process consists of utilizing a reverse phase emulsion (water-in-oil) to extract the ink, and then causing the emulsion to reverse phase to an oil-in-water emulsion which is easily washed from the stock. Such a procedure overcomes the difficulties of the methods now in use. The ink is readily extracted, since the product functions as a solvent, and removal after reversion of phase is facilitated because the original emulsion carries sufficient emulsifier to carry both the solvent and the extracted ink or pitch.

The novel product contains solvent, emulsifier, and electrolyte, and water. The following materials may be employed in such a product.

**Solvent.**—Any water-immiscible solvent may be employed, including petroleum distillates, coal tar distillates of all types, chlorinated solvents such as carbon tetrachloride, orthodichlorobenzene, trichloroethylene, etc. Kerosene is preferred due to its low cost, satisfactory solvent power, and relatively high flash point.

**Emulsifier.**—As emulsifiers, any of the group of soaps, mineral oil sulfonates, esters, glycerides, or the like may be used. Examples are sodium or potassium oleate, sodium salt of a mineral oil

sulfonic acid, diglycol oleate, mannan-mono-palmitate, mono-glyceryl oleate.

**Electrolyte.**—In order to form water-in-oil emulsions, it is usually necessary to have present an electrolyte which preferentially forms this type of emulsion. For this invention, it is necessary that this electrolyte be of such nature that upon addition of alkali its action is destroyed, and the emulsion reverses phase. Useful electrolytes include salts of bivalent and trivalent metals and certain organic acids. Examples are aluminum sulfate, potassium sulfate, magnesium sulfate, calcium chloride, ferric or ferrous sulfates, oxalic acid, acetic acid, citric acid, lactic acid, etc.

The treating or de-inking reagent, as applied to the pulp is the reverse phase (water-in-oil) emulsion. Such emulsions are relatively well known, and a few examples of such emulsions, particularly suitable for such use, follow:

*Example I*

|                                    | Weight percent |
|------------------------------------|----------------|
| Mineral oil sulfates (oil soluble) | 15.0           |
| Kerosene                           | 40.0           |
| Potassium aluminum sulfate         | 1.5            |
| Water                              | 43.5           |

*Example II*

|                                      | Weight percent |
|--------------------------------------|----------------|
| Oil soluble mineral oil sulfonates   | 7.5            |
| Water soluble mineral oil sulfonates | 2.5            |
| Kerosene                             | 40.0           |
| Epsom salt (magnesium sulfate)       | 2.0            |
| Water                                | 48.0           |

Other representative formulae which may be used are as follows:

*Example III*

|                                    | Weight percent |
|------------------------------------|----------------|
| Oil soluble mineral oil sulfonates | 10.0           |
| Kerosene                           | 40.0           |
| Epsom salt                         | 1.0            |
| Water                              | 49.0           |

*Example IV*

|                      | Weight percent |
|----------------------|----------------|
| Sodium oleate        | 8.0            |
| Carbon tetrachloride | 10.0           |
| Kerosene             | 30.0           |
| Epsom salt           | 2.0            |
| Water                | 50.0           |

*Example V*

|                                  | Weight percent |
|----------------------------------|----------------|
| Mineral oil sulfonates           | 10.0           |
| Coal tar solvent naphtha (xylol) | 50.0           |
| Oxalic acid                      | 1.0            |
| Water                            | 39.0           |

*Example VI*

|                      | Weight percent |
|----------------------|----------------|
| Diglycol oleate      | 7.0            |
| Kerosene             | 25.0           |
| Orthodichlorobenzene | 25.0           |
| Trisodium phosphate  | 3.0            |
| Water                | 40.0           |

The manufacture of the above emulsion consists essentially of the following: The solvent and emulsifier are mixed in one container; and the water and salt or acid, (electrolyte), in a second. With vigorous agitation the aqueous solution is added to the solvent solution, and stirring is continued until the product is made homogeneous.

In Example VI a formula is given which is set up on a basis unique as compared to preceding

Examples I to V inclusive. With Examples I to V inclusive, the change of phase is accomplished by added alkali as will be observed later. With Example VI, the alkali required for phase reversal is present, but inactive until the change is promoted by heating.

*De-inking and de-pitching procedure*

The following procedure is followed in using these emulsions: The stock in the beater, either waste paper or virgin pulp, is brought to a point where it is thoroughly wet-out and digested. The pH of the stock is lowered to below 6.5. A pH of 4.5 is preferred, although this is not essential. At this point the reverse-phase emulsion is added and allowed to mix intimately with the stock. Between 2 and 50 gallons of emulsion may be used for one ton of dry pulp, although the preferred quantity is between 10 and 20 gallons, depending upon the condition of the pulp to be treated. For de-inking waste paper, more emulsion is needed than for the removal of pitch.

After the emulsion has been thoroughly mixed with the stock and has dissolved the ink or the pitch, the stock is neutralized and rendered slightly alkaline with caustic soda, soda ash, trisodium phosphate or the like. Any pH above 7.0 is satisfactory after neutralization, although a pH of 8.0-8.5 is preferred. The contents of the beater may be heated to facilitate the reversion of phase, but this is not always essential. After the emulsion has reversed completely, it is washed from the stock in the usual manner.

When using a "self-reversing" emulsion such as that of Example VI, where sufficient alkali for phase reversal is incorporated in the formula, but remains inactive until the application of heat, the phase reversal will, of course, be accomplished simply by heating to a proper degree. With the emulsion of Example VI, the phase reversal will be accomplished by heating to about 160° F. to 180° F.

It will thus be seen that while the process here disclosed may make use of solvents and emulsifiers known and presently used for the same overall purpose, it makes use of those materials in a new and far more effective way, in that where pitchy materials, (and ink is such a pitchy material), must be dissolved, the reagent has a high capability of reaction in that it presents an external phase selectively capable of attacking the pitch and ink, yet, when it comes to removing the reagent, it has been converted to a highly water miscible state.

Certain comments are of interest. The operation may be conducted either in a beater or in a pulp digestor. It can be conducted more advantageously in a pulp digestor. Here a heavier pulp—more fibre and less water—is formed. This is advantageous in that when the emulsion is inverted by the addition of alkali a more concentrated oil-in-water emulsion results than if the operation is conducted in a beater with a less concentrated pulp. The more concentrated emulsions are more stable and are more easily washed from the pulp.

In formulae like that of Example VI care should be taken not to use them with pulps of very low pH since with such stocks the alkalinity of the formula upon heating may not be enough to overcome the acidity of the stock. Of course, where this condition is known to exist, proper adjustment of the electrolyte proportion in the formula can be made to take care of the unusual condition. Since most reworked stocks are not thus unusual, and since, even with virgin pulp,

when one is removing pitch, the recirculated "white water" tends to hold the acidity at optimum levels, this unusual condition does not often obtain.

In proportioning the amount of emulsion to be used, the concentration should be adjusted upon the basis of water present in stocks. With beater stocks, the proportions of 2 to 50 gallons per ton of dry pulp, preferred ranges being 10-20 gallons per ton should be used, and with more concentrated stocks these proportions should be adjusted with regard to the amount of water present to arrive at water/emulsion ratios of the same magnitude as those indicated for beater stocks.

We claim:

1. That method for the removal of pitchy materials from paper pulp stocks comprising the steps of contacting the stock while in a digested and acid condition with an invert emulsion of a solvent for such pitchy material to substantially dissolve the pitchy material therein, then changing the phase relationships of the emulsion and washing the emulsion, containing dissolved pitch, from the stock.

2. That method for the removal of pitchy materials from paper pulp stocks, comprising the steps of admixing with the wet-out, acid, and digested stock an emulsion of the water-internal type, comprising a water-immiscible solvent for

the pitchy material, an emulsion forming material, and an emulsion inverting electrolyte inactive under alkaline conditions, dissolving and removing said pitchy materials by the use of said invert emulsion, then causing reversion of the emulsion to a water-external type, and washing the emulsion and contained pitchy material from the pulp stock.

3. That method for the removal of pitchy materials from paper stocks comprising bringing the stock to a hydrogen ion concentration of below about 6.5, adding thereto a water-internal type of emulsion comprising a solvent agent for the pitchy material, substantially removing said pitchy material from said stock by the use of said emulsion, then bringing about reversion of the emulsion to the water-external type, and removing said emulsion and contained pitchy material from said stock.
- 10 4. That method for the removal of pitchy materials from paper stocks comprising bringing the stock to a digested and acid condition, adding thereto a water-in-oil emulsion stable under acidic conditions and agitating it with the stock to dissolve and remove pitchy material therefrom, then bringing the stock to an alkaline condition and inverting the emulsion to an oil-internal condition and washing the emulsion from the stock.

JOHN C. DEAN.  
ROY T. EDWARDS.